

Dec. 15, 1964

C. L. GOSS ET AL

3,161,227

## INFRARED GAS BURNER

Filed April 24, 1962



Fig. 1



Fig. 2



Fig. 3

INVENTORS  
CHARLES L. GOSS  
LEONARD C. LIPTAK

BY

Brown, Critchlow, Flick & Peckham  
ATTORNEYS.

1

3,161,227

## INFRARED GAS BURNER

Charles L. Goss and Leonard C. Liptak, Corning, N.Y.,  
assignors to Corning Glass Works, Corning, N.Y., a  
corporation of New York

Filed Apr. 24, 1962, Ser. No. 189,785  
8 Claims. (Cl. 158—99)

This invention relates to infrared gas burners and in particular it comprises novel structure including a mixing chamber and a burner plate on the surface of which nearly incandescent combustion takes place.

Infrared gas burners are known in the art and are exemplified by such United States patents as Burns et al., Number 1,896,236, Schwank, Number 2,775,294 and Schwank et al., Number 2,870,830. It will be noted that in the prior art much attention has been given to the provision of adequate mixing of the gas and air combustion mixture, and to avoiding the phenomenon termed flashback in which combustion takes place below the burner plate thereby stopping normal operation and in many cases destroying the complete burner.

Despite the efforts made in overcoming flashback and the like, our studies have shown that this problem remains in the art to a degree. Moreover, there are other problems that provide limitations on the effectiveness of these burners. For example, we have found that the available gas burners are characterized by a moderately limited temperature of operation. When temperatures of a higher level are experienced, fracture of the burner plates or separation from the supporting structure and destruction of the mixing chamber can occur.

It is, therefore, a primary object of the present invention to provide an infrared gas burner structure that can operate at a considerably higher temperature than gas burner structures presently available, that is characterized by thermal expansion characteristics such that its various parts fuse rather than fracture or separate from one another at excessive temperatures, that is easily prepared from inexpensive materials and with skills presently available in the art.

Another object is to provide a novel burner plate for a structure in accordance with the foregoing object.

These and other objects are attained in accordance with our discoveries by providing an infrared gas burner comprising a thin wall ceramic honeycomb cover or burner plate and a body portion defining a mixing chamber having a gas inlet and supporting structure for the cover plate. Each of the parts is composed of a low thermal expansion lithium aluminosilicate ceramic material and they are joined to one another with a foamed ceramic cement of low thermal expansion to result in an essentially unitary structure. With the parts having particular characteristics as indicated hereinafter, there results an infrared burner that can safely be operated at very high temperatures for extended periods, that will not fracture upon being repeatedly subjected to excessive temperatures or temperature changes, that is free from the propensity toward flashback and yet is economical and is easily produced.

The invention will be described in detail in conjunction with the attached drawings in which:

FIG. 1 is a top view, with part of the cover plate broken away, of an infrared gas burner of the present invention;

FIG. 2 is a sectional view of the infrared gas burner of FIG. 1 taken along line II—II; and

2

FIG. 3 is a perspective view of a part of an infrared gas burner of the invention.

Referring now to the drawings, a gas burner 3 in accordance with this invention is composed of a body member 10 having an integral or separately attached centrally disposed inlet tube 12 extending from one side. The top surface or cover plate of the gas burner 3 is a ceramic honeycomb structure and is indicated by the numeral 14. The cover member 14 is attached to the body 10 by means of a particular foamed ceramic cement indicated by the numeral 16 in the drawings. The tube 12 is not essential to the invention and can be omitted when not desired.

As will be noted in FIGS. 1 and 2, the inlet tube 12, when used, suitably extends into the body 10 terminating near its wall 18 that is opposite the wall 20 through which the tube enters. The zone 22 within body 10 between the cover member 14 and the bottom wall 26 comprises a mixing chamber where air and the fuel, such as natural gas, propane, butane, manufactured gas, town gas, or the like, thoroughly mix prior to passing upwardly through the cover member 14 for combustion. While body member 10 is shown as a generally dish-shaped structure, it should be understood that various other shapes and inlet tube orientations can be used without departing from the scope of the invention.

Characterizing features of the invention include the use of a particular honeycomb structure as the cover member, and the manner of joining the cover member or plate to the burner body. As is shown in the drawings, the honeycomb cover member 14 is characterized by a large number of unobstructed gas paths 30 that extend from the bottom surface 32 of the cover member through to its top surface 34. These unobstructed gas paths are defined and separated from one another by thin ceramic walls 36. By unobstructed, we mean that no structure exists within the gas flow paths that would prevent flow. The ceramic walls defining those flow paths can be arranged in triangular or polygonal shape as desired.

The cover honeycomb is attached to the body member 10 at the upper portion of the side walls of that member. That is accomplished by use of a low expansion ceramic cement 16 that is foamed in place and joins the cover plate 14 and body member 10 to a unitary structure.

In the use of a burner of the invention, a source of a gaseous fuel and air enter the burner body 10 through the inlet tube 12 or any other suitable inlet means. The fuel and air can be provided by sources connected to a mixing head that is attached to the inlet means, or the pressure of the fuel gas can be used with suitable means to aspirate air into the stream. Other procedures, none of which form any part of the invention, can be used as well. The gases enter the enlarged space 22 within the burner body 10 and thoroughly mix therein. For mixing purposes, the inlet tube can be designed so that the gases impinge on a wall of the body member 10, or baffles (not shown) can be included within the body to effect that object. The mixed gases then pass through the gas paths 30 in the cover plate to the upper surface where they are combusted, raising the surface of the plate to nearly incandescence. Any suitable conventional combustion initiator can be used as desired.

Ceramic honeycomb structures that are used for burner plates in accordance with the present invention have certain definite characteristics that are essential for proper operation and to provide the outstanding advantages

characteristic of the invention. The honeycomb, as well as the body member and the foaming cement, must be formed of ceramic materials sintered to a unitary structure and that provide a low coefficient of thermal expansion in the fired state. Ceramic materials that provide such a coefficient of expansion inherently have a high heat conductivity on the order of at least 0.0020 cal./sec. cm. °C. or higher. While a high heat conductivity generally would be considered disadvantageous, that property is not deleterious in the present invention but is compensated by the high specific heat and the thinness of the walls defining the honeycomb. The wall thickness is below a 0.01 inch and generally is in the range of 0.005 to 0.008 inch. Even thinner walls may be used if desired. As will be noted from the drawings, two walls come together to point contact at various locations in the honeycomb. At that point, the overall wall thickness may approach 0.02 inch. Such junctures, however, involve but a few percent (e.g., less than five percent) of the total and therefore are insignificant. The length of the gas flow passages, and therefore the thickness of the burner plate, must be at least 0.2 inch and preferably is at least 0.375 inch. Usually, the plate thickness does not exceed about three quarters of an inch.

The high specific heat of the ceramic of the honeycomb contributes to heat absorption whereby good infrared radiation is achieved, and is on the order of 0.20 calorie per gram or higher at 25° C. The high thermal conductivity tends to conduct heat away from the burner surface. Normally that would contribute to flashback, but it does not do so in our invention. The gas passages have a small cross-sectional area and accordingly gas velocity, for a given gas inlet pressure, is relatively high. Therefore, the gas abstracts the heat absorbed by or conducted along the thin walls, keeping the upstream portion of those walls at a low temperature and avoiding the tendency to flashback. For example, with a gas flow path having a cross-sectional area of one square millimeter, an inlet gas pressure of 4 to 7 inches of water and a wall thickness of 0.005 to 0.010 inch, a glowing zone results in the honeycomb burner plate that extends from its burning surface inwardly to about 0.06 inch. The temperature in that zone is on the order of 1500° to 1700° F. Immediately adjacent the glowing zone is a transition zone of about 0.01 to 0.03 inch in length over which the temperature varies from about 1500° F. at the edge of the glowing zone down to about 300° F. at the bottom or upstream limit of the transition zone. This gradient and the relatively cold upstream condition are brought about by the effective cooling action of the high velocity fuel mixture, resulting from the small cross-sectional area of the gas passage, flowing against the thin walls, the minimal mass of the walls permitting rapid heat removal.

The gas passages have an average port or cross-sectional area at the burning surface that does not exceed 0.006 square inch and preferably is below about 0.005 square inch. The gas passages or ports are, of course, uniformly distributed throughout the burner plate and their cross-sectional areas in the aggregate must provide at least 50 percent and preferably at least 60 percent of the total area of the burner plate surface. It has been found that these limitations are critical. For example, with a larger individual port area, the gas velocity for a constant gas input pressure would drop below the value necessary to counteract or offset the flame front velocity, i.e. the rate at which the flame will ignite fresh gas coming in contact with the flame. Furthermore, the lower gas velocity would not adequately cool the ceramic walls. Accordingly, a larger cross-sectional area for the ports would render the structure more subject to flashback.

When an open area less than 50 percent of the total surface area of the burner plate, for the standard commercial gas line pressures of about 4 to 7 inches of water, unduly high gas velocity through the gas paths would

result. That would blow the flame up off the burner surface and quite possibly extinguish it. In either instance, the upper portion of the ceramic walls would not absorb sufficient heat to cause the surface to radiate infrared wave lengths. In addition, with an open or port area that is less than 50 percent of the total burner surface and with ports of the size indicated, there would be an excessive amount of the area occupied by the ceramic walls which would have to be made larger, and therefore be relatively massive. In that instance, excessive heat absorption would occur and the ceramic would act as a flame arrestor.

An important advantage of the requirement for the large open area for the burner plates is that, for a given gas inlet pressure, it provides a greater heat input in consequence of the lessened pressure drop across the thickness of the burner plate. Accordingly, a greater volume of gas per unit of time is passed through the burner plate and burned with a correspondingly greater production of heat. This advantage results in the ability to provide smaller and more compact burner units to meet a given heat output requirement since the open area provides a greater total gas throughput and therefore a greater total heat production.

The very thin walls of the ceramic honeycomb that are necessary in producing suitable burner plates for this invention cannot be achieved by molding processes. To attain the strength in the green state necessary for a molding process would require far thicker walls. The thin walls of the honeycomb are not fragile, contrary to expectation. The low expansion lithium aluminosilicates sinter to a surprisingly strong and dense structure. Accordingly, operation to higher temperatures without mechanical destruction is possible. And this is achieved despite the severe thermal gradient to which this seemingly fragile structure is subjected.

Ceramic honeycomb bodies that serve as the burner plate in this invention and conform to the limitations stated can be prepared by several processes. For example, a pulverized ceramic material can be admixed with a suitable binder and then extruded to a ribbon form. The resulting ribbon can be further shaped, if desired, and assembled either by itself or with other ribbons of this material, to the desired honeycomb shape. The resulting assembly is then sintered to a unitary structure. Preferably, however, the ceramic honeycomb body is prepared by coating a suitable carrier with a mixture of a pulverized ceramic and a binder, crimping the resulting coated carrier and then assembling it to the desired shape alone or with another coated carrier that need not be crimped. The assembled body is then heated to a temperature sufficient to sinter it to a unitary structure as more fully detailed hereinafter. This latter procedure is, generally the process set forth in the co-pending application of Robert Z. Hollenbach, Serial Number 759,706, filed September 8, 1958, now Patent 3,112,184.

The purpose of the binder is to bond the unfired ceramic material to the carrier, to impart green strength to the coated carrier and to retain the formed unfired article in the desired shape after forming and prior to sintering. In order that the resultant article be essentially all ceramic material having a low coefficient of thermal expansion, it is preferred to use an organic binder, especially those that are heat curable or thermosetting that can be removed by decomposition and/or volatilization when the article is fired. Among the many materials having the requisite, well known characteristics of binders that can be used in the process are such natural materials as gum arabic, colophony and shellac and such synthetic organic resins as acrylate resins, methacrylate resins, alkyd resins, cellulose derivatives, coumarone indene resins, phenolic resins, polyamides, polyesters, resorcinol resins, styrene resins, terpene resins, urea resins,

vinyl resins, epoxy resins, chlorinated paraffins and melamine resins.

The purpose of the carrier is to provide support for the unfired coating to allow it to be formed to the desired shape prior to sintering the ceramic coating. Tea bag paper is a preferred carrier and a list of other suitable materials is disclosed in the aforementioned Hollenbach patent, to which reference can be made. Tea bag paper, as well as other organic film materials, substantially decompose upon firing and thus result in an article consisting almost entirely of ceramic material.

In order to produce a structure having characteristics suitable for an infrared burner plate in accordance with our discoveries, it is essential that ceramic materials be used that have a low coefficient of thermal expansion in the fired state on the order of about minus 10 to plus 20 times  $10^{-7}$  °C. over an extended temperature range. Suitable ceramic materials for the burner plate include lithium aluminosilicates such, for example, as glass or crystalline petalite and beta spodumene, glass-ceramics having a lithium aluminosilicate base and especially those made in accordance with Example 1 of United States patent to Stookey, Number 2,920,971, as well as mixtures of any of the foregoing materials. Petalite glass-ceramic mixtures generally include about 10 to 40 weight percent of the glass-ceramic and the remainder petalite. Beta spodumene-petalite mixtures usually contain about 1 to 4 parts of petalite for each 4 to 1 parts of beta spodumene. These materials normally are used in a particle size of about minus 200 mesh (Tyler) or finer, depending on the wall thickness desired in the resulting article.

Structures are assembled from ceramic coated carriers in a variety of ways, and the resulting structures are called honeycombs, a term which in this specification means a unitary body having a multitude of unobstructed gas paths of predetermined size and shape, each such gas path being defined by thin ceramic walls and extending between and terminating in opposed surfaces. These structures can be assembled from multiple layers of film corrugated with the same pattern with alternate layers laterally disposed a distance equal to half of the width of the individual pattern so that layers do not nest with each other. The honeycomb structure can also be formed from rolling alternate layers of crimped and uncrimped coated carriers until the desired shape is formed. The structure can also be formed by assembling to a stack alternate crimped and uncrimped coated carriers until the desired dimensions are attained. Since the minimum thickness for suitable burner plates (i.e. length of gas flow paths) is at least 0.2 inch, the structure is either formed in that size or a fired body is cut to the desired thickness. Other ways of assembling these honeycombs will be apparent to those skilled in the art.

The firing of the green structure or matrix, however formed, is accomplished in the normal manner for ceramic firing by placing the article in a furnace and heating it at a rate slow enough to prevent breakage up to a temperature high enough to cause the ceramic particles to sinter. While the firing schedule, including heating rates and sintering temperatures, will vary depending upon the ceramic material utilized, the size and shape of the article formed, and the atmosphere used, the details of such schedules are not critical and suitable conditions are readily determinable by one skilled in the art of firing ceramic articles.

The burner body member 10 and inlet tube 12 for use in the invention can be made by any of the techniques available in the ceramic and glass arts. For example, they can be cast from suitable ceramic mixtures, as by making a slip of the ceramic materials, casting the slip, and then firing to a unitary structure. They can also be formed of the suitable glass, ceramics by the conventional hot glass forming techniques well known in the art for these materials. If the inlet tube is separately formed, it can readily be joined to the body member 10 by use of the

foaming cements referred to hereinafter. As already noted, the burner body member must have a low coefficient of thermal expansion. Accordingly, it is made from one or more of the materials mentioned above as suitable in forming the honeycomb burner plate.

The heater body and honeycomb cover plate are joined to provide a unitary structure by use of a ceramic cement that will foam and readily bond those members and that has a low coefficient of thermal expansion in the foamed state. Cement for this purpose has a composition, by weight, of 1 to 16 percent of lead oxide, 1 to 15 percent of a flux, 1 to 6 percent of silicon carbide, 1 to 6 percent of  $\text{SO}_3$  and substantially all of the remainder, and at least about 70 percent of the total cement composition, a lithium aluminosilicate ceramic such as glass or crystalline petalite and beta spodumene, a glass-ceramic having a lithium aluminosilicate base such as that of Example I in the mentioned Stookey patent, as well as mixtures of any of the foregoing. Glass petalite is the preferred ceramic. Typical flux materials include the fluorides and oxides of magnesium, calcium, strontium, barium, zinc, cadmium, lead, lithium, sodium and potassium. Suitably a mixture of oxide and fluoride fluxes is used. The  $\text{SO}_3$  content of the batch is provided by, for example, a compound such as calcium sulfate, barium sulfate, strontium sulfate, magnesium sulfate, zinc sulfate, cadmium sulfate, lead sulfate, sodium sulfate, potassium sulfate or lithium sulfate. It will be apparent that the use of any of these compounds provides both the  $\text{SO}_3$  and an oxide flux. Lead sulfate, which also may be used, provides the essential lead oxide and  $\text{SO}_3$ . The cement is used by pouring it into the spaces between the parts to be joined and then firing the unit to a temperature of about 1050° to 1150° C. or more until foaming and sintering are complete. Thereafter, the unit is cooled to handling temperature.

The invention will be described further in conjunction with the following example in which the details are given by way of illustration and not by way of limitation.

In this example, a ceramic composition is made of 75 parts by weight of petalite and 25 parts by weight of a glass-ceramic having the following approximate composition, by oxide analysis, in weight per cent: 70 percent  $\text{SiO}_2$ , 13 percent  $\text{Al}_2\text{O}_3$ , 5 percent  $\text{TiO}_2$ , 3 percent  $\text{Li}_2\text{O}$ , 3 percent  $\text{MgO}$  and 1 percent  $\text{ZnO}$ . The composition is ball-milled to a minus 200 mesh (Tyler) particle size. A solution of the following composition is added to 2160 grams of the ceramic material in the ball mill:

|    |                          |
|----|--------------------------|
| 50 | 640 cc. of isopropanol   |
|    | 860 cc. of ethyl-acetate |
|    | 180 cc of Versamid 115   |
|    | 480 cc. Hysol 6111       |

Versamid 115 is the trade name of a thermoplastic polymer supplied by General Mills, Inc. It is prepared by condensation of polymerized unsaturated fatty acids, such as dilinoleic acid, with aliphatic amines such as ethylene diamine. Hysol 6111 is the trade name of an epoxy resin solution, supplied by Houghton Laboratories, Inc. containing 57 percent by weight of epoxy resin having a viscosity of about 2.5-4.0 poise at 25° C., an epoxide equivalent (grams of resin containing 1 g. chemical equivalent of epoxy) of  $595 \pm 50$ , and a melting range of 73-85°C.

The ceramic material and the binder are further ball-milled for about three hours to produce a uniform suspension. A porous natural cellulose paper, commonly known as 3½ pound tea bag paper, cut to a width of 4 inches is then dipped into the suspension and dried by heating to 120° C. for 2 minutes. The dried, coated paper is then heated to 180° C. and crimped to produce a pattern, taken in cross-section, in the shape of an isosceles triangle with legs about 0.07 inch long and an open base about 0.1 inch wide. The crimped, unfired, coated paper is rolled up simultaneously with a sheet of tea bag paper of the same width, which has been coated in the

same manner but not crimped, upon a 2-inch diameter reel until an annular cylinder with an outside diameter of about 23 inches is obtained. Preferably, the uncrimped coated paper is not dried prior to the roll-up operation, but this paper is dried by forcing air heated to about 120° C. through the channels of the annular cylinder as they are formed during the roll-up operation.

The unfired matrix body is then placed in a furnace chamber and heated in accordance with the following schedule:

| Temperature Range:    | Firing Rate   |
|-----------------------|---------------|
| Room Temp. to 700° C. | 350° C./hr.   |
| Hold at 700° C.       | 1 hour.       |
| 700° C. to 1220° C.   | Furnace rate. |
| Hold at 1220° C.      | 30 minutes.   |
| Cool to Room Temp.    | Furnace rate. |
| Refire to 1240° C.    | 300° C. hr.   |
| Hold at 1240° C.      | 7 hours.      |

Thereafter the matrix is cooled to handling temperature.

A body member as shown in the drawing is made from a ceramic composition as stated above. The ball-milled ceramic mixture is tempered with water to a slip consistency, and cast in an absorbent mold. After the cast article has developed strength by partial drying, the mold is removed and the body member is thoroughly dried by heating at 125° C. for 10 hours. Thereafter, it is fired at 1250° C. for 8 hours.

The body and a section of honeycomb, i.e. about  $\frac{3}{8}$  inch thick section sawed from the matrix, are assembled. Then a cement having the following composition, by weight, is used to join these members: 8.72 percent of zinc oxide, 1.3 percent of calcium fluoride, 3.46 percent of silicon carbide, 1.93 percent of  $\text{SO}_3$ , 6.81 percent of  $\text{PbO}$  and the remainder glass petalite. A batch of this cement composition is dispersed in a mixture containing 75 weight percent of butyl alcohol and 25 weight percent of toluene and is wet ball-milled to thoroughly mix the batch. This cement is poured in the annular spaces in the assembly. The resulting assembly is then placed in a furnace and raised to 100° C. at a rate of 2° C./min. After 2 hours at 100° C., the temperature is raised at 5° C./minute to 1150° C. and is held at 1150° C. for one hour and 15 minutes to permit the foaming action to be completed. It is then furnace cooled at a rate of 5° C./min. to handling temperature.

Ceramic infrared gas burners prepared as just described have been actually tested and have been found to be entirely satisfactory. Extended operation with the burning surface cycled at temperatures between room temperature and about 1100° C. did not adversely affect the structure, neither causing fracture nor separation of the cover from the body of the burner. As far as is known, no other ceramic burner for this purpose could successfully operate by cycling at temperatures between room temperature and about 1100° C. for any material period of time without destruction occurring.

From the discussion and description, it is evident that the present invention constitutes an important advance in the art of infrared gas burners. By this invention such burners are provided that can operate at higher temperatures for longer periods of time than other burners, yet the improved burners are more durable and safe to operate and are relatively inexpensive to produce. These outstanding advantages are largely the result of using the lithium aluminosilicate ceramics of low thermal coefficient of expansion, the provision of a truly unitary structure by reactively joining the cover and body member with the cement foamed in situ, and the formation of a dense, strong honeycomb with a resulting high thermal conductivity which is overcome by the use of thin walls thereby reducing heat conduction to and preventing ignition of the gas-air mixture at the inner burner plate surface.

In accordance with the provisions of the patent statutes,

we have explained the principle of our invention and have illustrated and described what we now believe to represent its best embodiment. However, it should be understood that, within the scope of the appended claims, the invention can be practiced otherwise than as specifically described.

We claim:

1. An infrared gas burner comprising a ceramic burner body member defining a mixing zone, inlet means through a wall of the body member for the introduction of air and fuel, a ceramic cover plate on said burner body member, and a foamed ceramic cement joining said cover plate and body member to one another providing a unitary structure, said cover plate comprising a thin walled ceramic honeycomb having a pair of opposed surfaces and a plurality of unobstructed gas passages extending between and terminating in those surfaces, the body member, cover plate and foamed cement all having a low and substantially similar coefficient of thermal expansion.
2. A gas burner according to claim 1 in which each gas passage has a cross-sectional area that is less than 0.006 square inch and the collected cross-sectional areas of the gas passages provide an open space of at least 50 percent of said surfaces.
3. A gas burner according to claim 2 in which the ceramic of the body member, the honeycomb and the cement comprises a lithium aluminosilicate.
4. A gas burner according to claim 2, in which the ceramic of the body member and the honeycomb comprises a lithium aluminosilicate and the composition of the cement is, by weight, 1 to 16 percent of lead oxide, 1 to 15 percent of a flux, 1 to 6 percent of silicon carbide, 1 to 6 percent of  $\text{SO}_3$  and the remainder a lithium aluminosilicate ceramic, said lithium aluminosilicate ceramic comprising at least 70 percent of the total cement composition.
5. An infrared gas burner comprising a ceramic burner body member defining a mixing zone, inlet means through a wall of the body member for the introduction of air and fuel, a ceramic cover plate on the burner body member, and a foamed ceramic cement joining the cover plate and body member to one another providing a unitary structure, the cover plate comprising a thin walled honeycomb having an inlet surface and an opposed combustion surface and a plurality of unobstructed gas passages uniformly distributed throughout the honeycomb and extending between and terminating in those surfaces, each gas passage having a cross-sectional area that is less than 0.006 square inch, the collected cross-sectional areas of the gas passages providing an open space at the combustion surface that is at least 50 percent of the total area of the combustion surface, the thickness of the walls of the honeycomb being below about 0.01 inch, the thickness of the honeycomb being at least 0.2 inch, the body member, cover plate and formed cement all having a low and substantially similar coefficient of thermal expansion.
6. An infrared gas burner according to claim 5, the cross-sectional areas of the gas passages and the thickness of walls of the honeycomb being such that the free space at the combustion surface is at least 60 percent of the total area of that surface, and the thickness of the honeycomb being at least 0.375 inch.
7. An infrared gas burner according to claim 6 in which the ceramic of the body member, the honeycomb and the cement comprises a lithium aluminosilicate.
8. An infrared gas burner according to claim 6 in which the ceramic of the body member and of the honeycomb comprises a lithium aluminosilicate and the composition of the cement is, by weight, 1 to 16 percent of lead oxide, 1 to 15 percent of a flux, 1 to 6 percent of silicon carbide, 1 to 6 percent of  $\text{SO}_3$  and the remainder a lithium aluminosilicate ceramic, said lithium aluminosilicate ceramic comprising at least 70 percent of the total cement composition.

silicate ceramic comprising at least 70 percent of the total cement composition.

References Cited in the file of this patent

UNITED STATES PATENTS

5

1,222,922 Bone et al. ----- Apr. 17, 1917  
1,896,286 Burns et al. ----- Feb. 7, 1933

1,939,476 Werner ----- Dec. 12, 1933  
2,920,971 Stookey ----- Jan. 12, 1960  
3,041,190 Griffith et al. ----- June 26, 1962

FOREIGN PATENTS

Canada ----- Aug. 29, 1961  
France ----- Aug. 27, 1956